

## UNITED STATES PATENT OFFICE

2,690,998

## METAL SOAP GREASE CONTAINING ALKALINE EARTH METAL PHENOLATE

John P. Dilworth and Charles H. Culnane, Fishkill, N. Y., and Harry V. Ashburn, deceased, late of Beacon, N. Y., by Evelyn L. Ashburn, administratrix, Beacon, N. Y., assignors to The Texas Company, New York, N. Y., a corporation of Delaware

No Drawing. Application April 18, 1951,  
Serial No. 221,742

11 Claims. (Cl. 252—42.1)

1

This invention relates to a lubricating grease composition, and particularly to such a composition which is inhibited against copper corrosion.

Lithium base lubricating grease compositions have found substantial use in aircraft controls and for other purposes where operation over a wide temperature range, and particularly operation at extremely low temperatures, is encountered. U. S. Patent No. 2,450,221, Ashburn, Barnett and Puryear, is typical of a superior lithium base grease of this type prepared from a lithium soap of a hydroxy fatty acid or the glyceride thereof, such as hydrogenated castor oil, and containing as the major proportion of the liquid lubricating base an oil soluble high molecular weight high boiling liquid aliphatic dicarboxylic acid ester within the lubricating oil viscosity range and possessing lubricating properties. As disclosed therein, the lithium soap may be formed from a major proportion of the hydroxy fatty acid or glyceride thereof, and a minor proportion of a saturated fatty acid, the grease containing a small excess of free fatty acid. Such greases have exceptional shear and texture stability over a wide temperature range and excellent low temperature properties.

While the lithium base greases of the aforesaid type have proved eminently satisfactory in service, the increased use of copper and copper alloys in certain applications, particularly in aircraft and artillery control instruments, has introduced an additional problem of rendering the grease non-corrosive to copper in long time service. For this purpose, U. S. Army Specification 2-134 has prescribed a rigorous copper corrosion test for qualification under this specification. In attempting to meet this specification, it has been found that corrosion inhibitors heretofore employed in greases are ineffective.

One of the principal objects of the present invention is to provide a lubricating grease which satisfactorily meets the copper corrosion test of U. S. Army Specification 2-134.

Another object of the present invention is to provide a lithium base grease which retains all the desirable properties of the previously known greases of this type, including shear and texture stability over a wide temperature range and excellent low temperature properties, and at the same time is effectively inhibited against corrosion of copper and copper alloys in long time service.

In accordance with the present invention, the foregoing objects have been attained by incorpo-

rating in the grease about 0.25 to 5% by weight of an oil-soluble alkaline earth metal salt of an alkyl phenol compound selected from the group consisting of alkyl phenols having a total of 10 to 30 carbon atoms in the alkyl substituents on each benzene nucleus, and the corresponding alkyl phenol sulfides. Salts of this type have heretofore been suggested as detergent additives for mineral lubricating oils; but it was entirely unexpected that such salts would function in the present greases as copper corrosion inhibitors, since this action is completely remote from detergency.

The alkaline earth metal salts which are effective copper corrosion inhibitors for purposes of the present invention, are prepared from the alkyl phenols or the corresponding sulfides thereof having the structural formula



where R is an alkyl group containing 5 to 30 carbon atoms, n represents the number of alkyl substituents on each benzene nucleus and is generally 1 or 2 with the proviso that the total number of carbon atoms of the alkyl substituents on each benzene nucleus is at least 10, and x is either 1 or 2. The alkaline earth metal salts may be either normal salts wherein the alkaline earth metal completely neutralizes the OH groups of 2 molecules of the alkyl phenol, producing the compound having the formula



where M represents the alkaline earth metal, or may be the basic salt having the formula



when formed from the alkyl phenol. The corresponding normal alkaline earth metal salt formed

from the alkyl phenol sulphide is represented by the formula



while the basic salt has the formula



These various compounds may be prepared in known manner by the alkylation of a phenol or phenol sulfide with a selected olefin or olefin polymer of the proper chain length, namely from 5 to 30 carbon atoms, in the presence of a suitable alkylation catalyst, such as HF,  $\text{BF}_3$  and the like. The olefin polymer is preferably prepared by polymerizing propylene under pressure, using for example a  $\text{BF}_3 \cdot \text{H}_2\text{O}$  catalyst. Likewise butylene polymer can be used. Depending upon the conditions of the alkylation, the phenol or phenol sulfide may be mono- or di-alkylated. Where a lower molecular weight olefin, such as amylene is employed for alkylation, the phenol or phenol sulfide is dialkylated to provide a total of at least 10 carbon atoms in the substituent alkyl groups. Where a high molecular weight olefin is employed, such for example as a propylene polymer fraction having olefins of 15 to 30 carbon atoms in the molecule, the product is generally monoalkylated. In addition to simple phenol, other monohydroxy mononuclear aromatic compounds having the hydroxyl group attached to the ring can be employed as the starting material, such for example as the cresols, xylenols and other alkyl phenols, as well as other corresponding sulfides. In the following description and claims, all of these various alkylated compounds will be referred to as alkyl phenols or alkyl phenol sulfides.

The foregoing alkyl phenols or alkyl phenol sulfides, in solution in a suitable aromatic solvent, such as toluene, are then reacted with the alkaline earth metal compound to produce the corresponding alkaline earth metal salt. Any of the alkaline earth metals, including calcium, barium, strontium and magnesium can be employed, although barium and magnesium are generally preferred. In the manufacture of a magnesium alkyl phenolate, for example, the alkyl phenol in toluene solution may be reacted with magnesium methylate dissolved in excess methyl alcohol at a temperature of about 40-50° C., using slightly less than  $\frac{1}{2}$  mol of the magnesium methylate per mol of the alkyl phenol. The temperature is then increased and the methyl alcohol distilled off. The resulting toluene solution of magnesium alkyl phenolate, which is the normal salt represented by Formula No. 2 above, is filtered while hot; and then sufficient mineral lubricating oil, such as a distillate oil having an SUS viscosity at 100° F. of about 300, is added to produce an ultimate 25 to 50% concentrate of the magnesium alkyl phenolate in the lubricating oil. The toluene solvent is then stripped from the lubricating oil concentrate.

In preparing a basic alkaline earth metal salt of the foregoing alkyl phenols or alkyl phenol

sulfides, the latter are preferably reacted with a substantial excess of an aqueous solution of a water soluble alkaline earth metal salt. For example, in preparing a basic barium alkyl phenolate, an aqueous solution of barium chloride with the latter in excess of that required for neutralization is added to a lubricating oil solution of the alkyl phenol. The reaction mix is subjected to steaming with agitation for a substantial period of time, such as about 1-4 hours. Following separation of the aqueous phase, the lubricating oil solution of the basic barium alkyl phenolate is washed and then heated to remove residual mixture to obtain a lubricating oil concentrate of the desired additive in about 25-50% concentration. The basic salts may also be prepared by reacting an oil solution of the alkyl phenol or alkyl phenol sulfide with a methanol solution of an excess of barium hydroxide, and then removing the methanol.

Typical compounds prepared as outlined above and which are useful for purposes of the present invention are barium diamyl phenol monosulfide, barium diamyl phenol disulfide, basic barium cardanolate formed from hydrogenated cardanol, magnesium alkyl phenolate wherein the alkyl group contains from 15 to 30 carbon atoms and is preferably  $\text{C}_{18}$  to  $\text{C}_{22}$ , and similar compounds of the other alkaline earth metals. Instead of preparing the alkyl phenol or alkyl phenol sulfide by alkylation as described above, suitable alkyl phenols containing at least 10 carbon atoms in the alkyl substituents on each benzene nucleus can be used, such as the hydrogenated cardanol as specified above.

The above described alkaline earth metal salts of alkyl phenols or the corresponding alkyl phenol sulfides may be employed in lithium base greases formed from any saturated fatty material, such as the conventional saturated fatty acids or glycerides thereof, to provide copper corrosion inhibition.

Preferably, the lithium base greases formed from hydroxy fatty acids or their corresponding glycerides, such as hydrogenated castor oil, are employed to obtain the improved shear and texture stability. Suitable types of soap-forming hydroxy fatty acids and glycerides thereof are disclosed in said Patent No. 2,450,221. While the soap-forming hydroxy fatty acids or their glycerides may be used as the sole acidic component of the lithium soap, they may be blended or combined with the conventional saturated fatty acids or fats in such proportions that at least 50% of the total acidic component is comprised of the hydroxy fatty acids or glycerides thereof. In general, any of the recognized fatty acid materials normally used in grease manufacture may be employed providing they are essentially saturated in character. These fats and fatty acids include mixtures of fatty acid glycerides found in naturally occurring fats and oils, together with fractionated components thereof. The fatty acids may be a mixture of acids split off from these fats or prepared by hydrogenation of fish oils, or the individual acids themselves. Very satisfactory results are secured by employing as the saturated fatty material for the formation of the lithium soap a mixture of about 60-80% of hydrogenated castor oil or 12-hydroxy stearic acid, with 40-20% of a saturated fatty acid such as stearic acid. The grease may contain about 10-30% by weight of the lithium soap.

In order to obtain the improved wide temperature range and low temperature properties,

the liquid lubricating base of the lithium grease composition is preferably formed of a major proportion of a synthetic oleaginous lubricating compound or condensation product, many types of which are now known in the art. Very satisfactory synthetic lubricants of this character are represented by the high molecular weight high boiling liquid aliphatic dicarboxylic acid esters which are within the lubricating oil viscosity range and possess lubricating properties. The compounds within this particular class are the esters of such acids as sebacic, adipic, pimelic, azelaic, alkenyl succinic, alkylmaleic, etc. The esters thereof are preferably the aliphatic esters and particularly the branched chain aliphatic diesters. Specific examples of the preferred oleaginous compounds are di-2-ethyl hexyl-sebacate, di-2-ethyl hexyl azelate, di-2-ethyl hexyl adipate, di-sec-amyl sebacate, di-2-ethyl hexyl alkenyl succinate, di-2-ethoxyethyl sebacate, di-2-(2'-methoxyethoxy) ethyl sebacate, di-2-(2'-ethyl butoxy) ethyl sebacate, di-2-butoxy ethyl azelate, di-2-(2'-butoxy ethoxy) ethyl alkenyl succinate, etc.

These oleaginous compounds may be used as the sole oil component of the grease or they may be blended with a mineral lubricating oil. Where a blend is employed, and low temperature properties are required, the mineral lubricating oil is preferably a light refined distillate mineral lubricating oil, such as a naphthene or paraffin base distillate, having an SUS viscosity at 100° F. of about 50-130 and preferably about 100 secs. The mineral lubricating oil will generally constitute less than 50% of the blend, and ordinarily about 40-20% thereof. The mineral lubricating oil blend is advantageous where the lithium soap is formed in situ. In such case, the saponification of the fatty material with the lithium hydroxide and dehydration of the resulting soap are conveniently carried out in the presence of a portion of the mineral lubricating oil, and the synthetic lubricant together with the additives employed in the grease are then added following dehydration and as 45 the agitated soap mix cools.

The following examples are given to illustrate the present invention:

#### EXAMPLE 1

A lithium base grease was prepared from a fatty material consisting of about 75% by weight of hydrogenated castor oil and 25% by weight of stearic acid. The lubricating base used was a mixture of about 75% by weight of di-2-ethyl hexyl azelate with about 25% by weight of a paraffin base mineral lubricating oil having an SUS viscosity at 100° F. of about 100. The method of preparation involved charging a steam heated kettle with the required amount of 10.3% lithium hydroxide solution together with a small amount of water, the hydrogenated castor oil and a small proportion of the paraffin base mineral lubricating oil, the latter being less than the amount of hydrogenated castor oil and generally about 1/2 to 2/3 of the latter. The kettle contents were held at 170-190° F. for about 4 hours with agitation, and then the stearic acid was added and the temperature maintained with stirring for another 1-2 hours to complete saponification. Following saponification, a 25% concentrate of an octyl methacrylate ester polymer in a mineral lubricating oil, which is sold commercially by Rohm and Haas under the name "Acryloid HF-600," was 65

added in an amount to provide 2% by weight of the concentrate in the final grease composition. The feature of adding methacrylate ester polymers of this type to a lithium base ball 5 and roller bearing grease for the purpose of noise suppression in bearings operated at high speeds is disclosed and claimed in the copending application of Dilworth, Finn and Puryear, Serial No. 220,538, filed April 11, 1951, now Patent No. 2,666,033. The saponified mix was then heated with stirring at 290° to 330° F. for about 4 hours to effect dehydration. The balance of the mineral lubricating oil was then added with stirring as the kettle contents cooled down to 15 about 280° F. The di-2-ethyl hexyl azelate was then slowly added with stirring as the mix continued to cool to about 220° F. Phenyl alphanaphthylamine in an amount of about 0.5% by weight based on the grease was then added as 20 an oxidation inhibitor, and a small amount of a dye was introduced. The resulting base grease was drawn at a temperature below 200° F. The resulting base grease had the following calculated composition:

|                                          | Weight percent |
|------------------------------------------|----------------|
| Lithium soap of hydrogenated castor oil  | 12.7           |
| Lithium stearate                         | 4.4            |
| Excess LiOH                              | 0.2            |
| Glycerine (from saponification of hydro- |                |
| genated castor oil)                      | 1.3            |
| Paraffin base lubricating oil            | 19.7           |
| Di-2-ethyl hexyl azelate                 | 59.2           |
| Phenyl alphanaphthylamine                | 0.5            |
| "Acryloid HF-600"                        | 2.0            |
| Dye                                      | 0.0027         |

To different portions of the foregoing base grease, various amounts of barium diamyl phenol sulfide, which is sold commercially by the Enjay Company, Inc. as "Paranox 56," were added as 40 shown in samples 2 and 3 in the following Table I. The said greases were then subjected to the copper corrosion test of the 2-134 specification with the results as shown in the table.

Table I

| Additive Wt. Percent | 2-134 Cu Corrosion Test |                     | Rating              |
|----------------------|-------------------------|---------------------|---------------------|
|                      | Copper                  | Grease              |                     |
| 50                   |                         |                     |                     |
| 1. Base Grease       | Grey stain              | Pink discoloration. | Fail.               |
| 2. Base Grease +1%   | Very slight stain.      | No change.          | Pass.               |
| 3. Base Grease +3%   | Clean                   | do                  | Do.                 |
| 4. Base Grease +1%   | Slight grey stain.      | do                  | Borderline to Pass. |
| 5. Base Grease +0.7% | Clean                   | do                  | Pass.               |
| 6. Base Grease +0.4% | do                      | do                  | Do.                 |
| 7. Base Grease +3.0% | do                      | do                  | Do.                 |
| 55                   |                         |                     |                     |
| 60                   |                         |                     |                     |

|                                                                     |       |
|---------------------------------------------------------------------|-------|
| (1), (2) and (3) Free alkali (LiOH)                                 | 0.09% |
| (4) Free fatty acid (oleic)                                         | 0.23% |
| (5) Free alkali (LiOH)                                              | 0.10% |
| (6) Free alkali (LiOH)                                              | 0.08% |
| (7) Prepared with di-2-ethyl hexyl sebacate—Free fatty acid (oleic) | 0.26% |

The 2-134 corrosion test of the foregoing table was run by placing a copper strip in a Norman-Hoffman bomb so as to be partially immersed in the sample of the grease under test, and then maintaining the bomb under oxygen pressure (110 pounds per sq. in. initial pressure) at 210° F. for 20 hours. During that period, no pressure drop due to oxygen absorption must occur. Then, at the completion of the 20-hour

period, both the sample of grease and copper strip are inspected. In addition to the requirement for no pressure drop during the test, there must be no more than a very faint stain on the copper strip and no more than a slight stain on the grease in order to be rated as passing. Slightly inferior products which do not merit a full "pass" rating are given a rating of "borderline to pass" where there is no more than a light stain on the grease and no pressure drop; and a rating of "borderline to fail" where there is a stain on the copper with or without a stain on the grease and no pressure drop. All other results are rated as "fail."

Since the foregoing greases of Table I, including the base grease of sample 1 which contained no corrosion inhibitor, all were compounded with about 0.5% by weight of the effective oxidation inhibitor phenyl alpha-naphthylamine they all satisfactorily met the requirement for no pressure drop during the test, and this item is not separately listed in the table.

Samples 1-3 inclusive of the foregoing table represent the base grease of Example 1, and the base grease compounded with 1% and 3% respectively of "Paranox 56." As will be noted from the calculated composition of the base grease, a calculated excess of 0.2% by weight of lithium hydroxide was employed in preparing this grease; and, as shown by Table I the greases of samples 1-3 analyzed to a free alkali content, calculated as lithium hydroxide, of 0.09%. It is to be noted that the base grease of sample 1 produced a grey stain on the copper strip and a pink discoloration on the grease, and thus failed the test. Samples 2 and 3 containing the "Paranox 56" successfully passed this rigorous copper corrosion test. In this connection, and as disclosed in the copending application of George W. Eckert Serial No. 210,096, filed February 8, 1951, now Patent No. 2,610,946, recognized copper corrosion inhibitors which are effective in other relationships are completely ineffective for purposes of the present invention. It was entirely unexpected that a material, such as an alkaline earth metal salt of an alkyl phenol sulfide, which is recognized as a detergent additive for lubricating oils, such as motor oils, but not as an anti-corrosive, should be effective as a copper corrosion inhibitor in the new environment of a lithium base grease.

In the aforementioned Eckert application, the use of a different type of copper corrosion inhibitor, namely a basic alkaline earth metal sulfonate, in a lithium base grease of this character is disclosed and claimed; and, further, it is pointed out that the grease should be prepared to a calculated excess alkalinity in order for this different type of copper corrosion inhibitor to be uniformly effective in the said 2-134 test. Samples 4-7 of the foregoing Table I show that this requirement of excess alkalinity is obviated by the copper corrosion inhibitors of the present invention. Thus sample 4 represents a grease prepared in accordance with Example 1 above except that a slight excess of stearic acid was used so that the grease analyzed to a free fatty acid content, calculated as oleic, of 0.23% by weight. As shown, 1% of "Paranox 56" in this grease gave a "borderline to pass" rating in the 2-134 copper corrosion test. Sample 7 of Table I represents a grease prepared in accordance with Example 1 above, except that di-2-ethyl hexyl sebacate was employed as the major portion of the lubricant base instead of

the corresponding azelate, and also an excess of stearic acid was again used in the formulation. 3% of "Paranox 56" in this particular grease gave a clear pass rating. Samples 5 and 6 of Table I were prepared in accordance with Example 1 above, using a calculated excess of lithium hydroxide of 0.3% and 0.2% respectively. It will be noted that as little as 0.4% by weight of "Paranox 56" in this grease gave a "pass" rating.

1164 gm. (3 mols) of alkyl phenol averaging C<sub>21</sub> alkyl group and 4 liters of dry toluene were charged to a 12 liter 3-neck flask fitted with a stirrer, thermometer, and condenser with a water trap. The materials were heated to toluene reflux temperature and the water present removed by means of the trap. The contents of the flask were cooled to about 40-50° C. and 36.4 gm. (1.5 mols) magnesium added slowly as magnesium methylate dissolved in approximately 1.5 liters of absolute methyl alcohol. The heat was gradually increased to the reflux temperature of methyl alcohol and the alcohol was removed by means of the trap. The temperature was then increased to the boiling point of toluene (230° F.). The solution was filtered through super cel Hy Flo and 3575 gm. 300 Pale Oil were added to the filtrate (sufficient pale oil to produce a 25% concentrate of additive after removing the toluene). The toluene was then removed by distilling in a Claisen-type distillation apparatus using a water aspirator. 4629 gm. of product was obtained. The product was heat treated by heating at 250° F. for 16 hours with stirring.

The foregoing concentrate of magnesium alkyl-21 phenolate (designated "MP-21") was blended into different portions of the base grease of Example 1 above to provide 1% and 3% respectively of the MP-21 on the weight of the grease, and the resulting grease compositions subjected to the 2-134 copper corrosion test with the satisfactory results shown in the following Table II:

Table II

| 50                            | Additive Wt. Percent | 2-134 Cu Corrosion Test |                | Rating |
|-------------------------------|----------------------|-------------------------|----------------|--------|
|                               |                      | Copper                  | Grease         |        |
|                               |                      | Clean.....              | No change..... |        |
| 1. Base Grease +1% MP-21..... |                      | Clean.....              | No change..... | Pass.  |
| 2. Base Grease +1% MP-21..... |                      | do.....                 | do.....        | Do.    |

EXAMPLE 3

1128 gm. (4 mols) of hydrogenated cardanol and 2610 gm. of 300 pale oil were charged to a 3-neck 12 liter flask fitted with a stirrer, thermometer, and water trap. The flask was heated to 50° C. to dissolve the cardanol and a mixture of 752 gm. (4 mols plus 10%) of anhydrous barium hydroxide and 4 liters of absolute methanol was added. The temperature was increased slowly up to the boiling point of the alcohol and the alcohol was removed from the flask by means of the trap. The temperature was then increased to 160° C., removing water by means of the trap. The reaction mixture was then allowed to cool, dissolved in benzene and filtered through filter cel. The benzene was removed by distillation and sufficient 300 Pale Oil was added to bring the mixture to 25% concentration of active material. This required about 2610 gm. 5240 gm. of product was obtained.

The foregoing basic barium cardanolate concentrate was blended into the base grease of Example 1 above, and the resulting blended grease compositions subjected to the 2-134 copper corrosion test with the satisfactory results as shown in the following Table III:

Table III

| Additive Wt. Percent                     | 2-134 Cu Corrosion Test |             | Rating |
|------------------------------------------|-------------------------|-------------|--------|
|                                          | Copper                  | Grease      |        |
| 1. Base Grease +1% Basic Ba Cardanolate. | Clean                   | Slight Pink | Pass.  |
| 2. Base Grease +3% Basic Ba Cardanolate. | do                      | No Change   | Do.    |

In addition to passing the rigorous 2-134 copper corrosion test, the greases of the present invention also satisfactorily pass the different copper corrosion test of Government Specification AN-G-25.

While the additives of the present invention have been specifically described above in connection with lithium base greases because these are representative of the type generally employed for specialty wide temperature range, and particularly low temperature service, it is to be understood that the invention is not limited thereto. Rather, the invention is also applicable to the improvement of the copper corrosion properties of other metal base greases, including those of sodium, calcium, aluminum, barium, and mixed base greases. For example, a grease comprising an oleaginous liquid lubricating base, such as a mineral lubricating oil or a synthetic lubricant base or mixture thereof, thickened to a grease-like consistency with about 10-30% of calcium 12-hydroxy stearate, may have added thereto for copper corrosion inhibition about 0.25-5% by weight of a phenolate or phenol sulfide of the type described above. The invention is particularly applicable to various metal base greases wherein the soap-forming fatty material of the metal soap consists of at least 50% by weight of hydroxy fatty acids or the glycerides thereof, such as 12-hydroxy stearic acid and hydrogenated castor oil.

It will be understood that the grease of the present invention may also contain other additives in small proportions which are compatible with the essential ingredients and do not interfere with the desirable properties thereof. Such additional additives include extreme pressure or lubricity agents, such as dibenzyl disulfide and triresyl phosphate, materials for improving resistance in the salt spray humidity cabinet test, such as sorbitan mono-oleate, and the like.

Obviously many modifications and variations of the invention, as hereinbefore set forth, may be made without departing from the spirit and scope thereof, and therefore only such limitations should be imposed as are indicated in the appended claims.

We claim:

1. A lubricating grease composition comprising as the essential constituents an oleaginous liquid lubricating base as the major constituent, about 10-30% by weight of a lithium soap of a saturated soap-forming fatty material, said grease normally being corrosive to copper, and from 0.25 to 5% by weight based on said composition of an oil-soluble alkaline earth metal salt of an alkyl phenol having a total of 10 to 30 carbon atoms in the alkyl substituents on each benzene nucleus, said salt being in sufficient proportion

to enable said grease composition to pass the copper corrosion test of U. S. Army Specification 2-134.

2. A lubricating grease composition according to claim 1, wherein said salt is a magnesium alkyl phenolate.
  3. A lubricating grease composition according to claim 1, wherein said salt is a basic barium alkyl phenolate.
  - 10 4. A lubricating grease composition comprising as the essential and at least major proportion of the lubricating base an oil-soluble high molecular weight high-boiling liquid aliphatic dicarboxylic acid ester within the lubricating viscosity range and possessing lubricating properties, sufficient lithium soap of soap-forming fatty material to thicken said lubricant base, said soap-forming fatty material consisting of more than 50% by weight of a hydroxy soap-forming fatty material selected from the group consisting of hydroxy fatty acids and hydroxy fatty acid glycerides, said grease normally being corrosive to copper, and from 0.5 to 3% by weight based on said composition of an oil-soluble alkaline earth metal salt of an alkyl phenol having a total of 10 to 30 carbon atoms in the alkyl substituents on each benzene nucleus, said salt being in sufficient proportion to enable said grease composition to pass the copper corrosion test of U. S. Army Specification 2-134.
  - 15 5. A lubricating grease composition according to claim 4, wherein said salt is magnesium C<sub>18</sub> to C<sub>25</sub> alkyl phenolate.
  - 20 6. A lubricating grease composition according to claim 4, wherein said salt is basic barium cardanolate.
  - 25 7. A lubricating grease composition comprising as the lubricant base a mixture of substantial proportions each of mineral lubricating oil and a branched chain aliphatic diester of a dicarboxylic acid selected from the group consisting of sebacic, azelaic and adipic acids, with said diester being in major proportion of the said mixture, about 10-30% by weight based on the composition of lithium soap of a mixture of a major proportion of hydrogenated castor oil and a minor proportion of stearic acid, said grease normally being corrosive to copper, and from 0.5 to 3% by weight based on said composition of an oil soluble alkaline earth metal salt of an alkyl phenol having a total of 10 to 30 carbon atoms in the alkyl substituents on each benzene nucleus, said salt being in sufficient proportion to enable said grease composition to pass the copper corrosion test of U. S. Army Specification 2-134.
  - 30 8. A lubricating grease composition according to claim 7, wherein said salt is magnesium C<sub>18</sub> to C<sub>25</sub> alkyl phenolate.
  - 35 9. A lubricating grease composition according to claim 7, wherein said salt is basic barium cardanolate.
  - 40 10. A lubricating grease composition consisting essentially of the following constituents in the approximate percentages by weight:
- |                                                                                                                                           |         |
|-------------------------------------------------------------------------------------------------------------------------------------------|---------|
| 65 Di-2-ethyl hexyl sebacate                                                                                                              | 50-85   |
| Lithium soap of a 2:1 to 4:1 weight mixture of hydrogenated castor oil and stearic acid                                                   | 10-30   |
| 70 Phenyl alpha naphthyl amine                                                                                                            | 0.3-1.0 |
| Alkaline earth metal salt of an alkyl phenol containing a total of 10 to 30 carbon atoms in the alkyl substituents on the benzene nucleus | 0.5-3.0 |
| 75 Mineral lubricating oil                                                                                                                | Balance |

11. A lubricating grease composition comprising as the essential constituents an oleaginous liquid lubricating base as the major constituent, about 10-30% by weight based on said composition of a metal soap of a soap-forming fatty material, said soap-forming fatty material consisting of at least 50% by weight of a hydroxy fatty material selected from the group consisting of hydroxy fatty acids and the glycerides thereof, said grease normally being corrosive to copper, and from 0.25 to 5% by weight based on said composition of an oil-soluble alkaline earth metal salt of an alkyl phenol having a total of 10 to 30 carbon atoms in the alkyl substituents on each benzene nucleus, said salt being in sufficient proportion to enable said grease composition to pass the copper corrosion test of U. S. Army Specification 2-134. 15

References Cited in the file of this patent

UNITED STATES PATENTS

| Number    | Name          | Date           |
|-----------|---------------|----------------|
| 2,351,384 | Woods         | June 13, 1944  |
| 2,362,289 | Mikeska       | Nov. 7, 1944   |
| 2,362,292 | McNab         | Nov. 7, 1944   |
| 2,397,956 | Fraser        | Apr. 9, 1946   |
| 2,409,303 | Morris et al. | Oct. 15, 1946  |
| 2,450,222 | Ashburn       | Sept. 28, 1948 |
| 2,483,505 | Rogers et al. | Oct. 4, 1949   |
| 2,518,379 | Rogers et al. | Aug. 8, 1950   |
| 2,610,982 | Hutcheson     | Sept. 16, 1952 |